

## UNITED STATES PATENT OFFICE

1,974,714

COMPOUND FOR PREPARING MATRICES  
FOR PRINTING PURPOSESRichard Junghänel and Hans Gross, Munich,  
GermanyNo Drawing. Application September 23, 1930,  
Serial No. 483,966. In Germany May 19, 1930

4 Claims. (Cl. 91—68)

Our invention relates to matrices such as are used in the manufacture of stereotype and other printing plates. More particularly, our invention relates to the process of manufacturing matrices which is performed as follows:

The surface of a base plate is treated mechanically by grinding or the like, so as to render it smooth and uniform and this mechanically treated surface is then treated with an impregnating compound containing a filler for the pores of the base plate and an adhesive. To the surface so treated and impregnated, a coating compound is applied which is allowed to dry, whereupon the matrix is treated mechanically, i. e. ground or polished, etc., to render its surface smooth and uniform.

According to our invention, the plate is treated with an impregnating and a coating composition, and the impregnating composition is so prepared as to effect a firm binding of the coating composition to the matrix.

The material of the matrices which serves as the base may be cardboard, asbestos, vegetable fibre, and a great variety of other suitable materials. This material is molded into thin sheets or boards.

Compounds of various compositions have already been suggested for coating the sheets or boards, but all such compounds are more or less unsatisfactory.

As is known, the types, stereotype plates, or electrotypes from which any number of prints is obtained by means of the matrices, are applied to the surface of the matrix after it has been slightly moistened so that the projecting portions of the original are impressed into the surface of the base. From the matrix thus obtained a stereotype plate is cast, usually in lead.

There are two methods of performing the molding operation, cold molding and hot molding. Cold molding is generally preferred on account of its more rapid performance, which is particularly important for automatic casting machines but the matrices in order to be suitable for cold molding must possess particular properties in order to fulfil the requirements of modern practice.

The processes of manufacturing such matrices which have been applied in practice, or have been described in literature, do not come up to all these requirements and therefore produce unsatisfactory matrices the defects of which have never been eliminated. Such defects are partly of a technical character but the principal defect is that it was impossible heretofore to obtain a

clear reproduction of pictures by the stereotype process, particularly for newspapers, in which low quality paper is used.

The causes of such defective reproductions are the more or less coarse texture of the material of the matrix and the unsuitable properties and limited durability of the coating compounds. It has been attempted to obtain better results by hot molding but clearly defined prints have not been obtained in this manner. In addition, the unfavorable operating conditions of the hot molding process, high pressure and elevated temperature, cause rapid wear of the expensive types, stereotype plates or electrotypes from which the matrices are copied.

Since cold molding is preferable in view of rapid production, which is particularly important for illustrated daily papers, a matrix in order to fulfil all requirements of modern practice, must be adapted to be molded by the cold process, and notwithstanding the short time available for performing the process the matrix must be of such a character that it will copy the finest impressions while at the same time possessing a high covering power and resiliency and being resistive to the heat of the liquid metal. The matrix must not be damaged anywhere, and particularly, in the case of a coated matrix, its material must nowhere be exposed, even at the most delicate points.

A matrix prepared according to our invention will stand the casting of a great number of stereotype plates in a modern automatic casting machine, and flat plates as well as arched plates such as are used in rotary printing machines, may be cast from the matrices with equal facility.

A matrix prepared according to our invention is practically free from defects. Autotype plates obtained from such a matrix will yield the finest and most clearly defined reproductions.

It is further possible to use a matrix prepared according to our invention, for producing therefrom other matrices in the same manner as the original matrix has been manufactured. In other words instead of casting a stereotype from the original matrix, a negative matrix is prepared from a matrix according to our invention by applying to such finished matrix a matrix which has been treated with the impregnating and coating compositions in the manner described. A matrix obtained in this manner is ready for immediate use as a printing plate.

In the manufacture of matrices according to our invention, the impregnating composition re-

ferred to below is either intimately mixed with the material of the matrix, or a sheet of card-board, asbestos board or the like is prepared from the material, without previous admixture of our 5 composition, ground at one of its faces, or at both faces, so as to remove any irregularities of its surface and any variations of its thickness. In this case the face of the matrix thus prepared is impregnated with a suitable liquid composition, which may for instance consist of 5 litres 10 water, 200 grammes glue, 70 grammes wax, 10 grammes nitric acid and 100 grammes suspended metal powder. The impregnating composition fills the pores of the base material and thereby 15 prevents rapid and unequal absorption of the liquid constituents of the coating compound which is subsequently applied to the impregnated surface, for fibrous material of the kind referred to has strong but unequally distributed 20 absorbing capacities. Apart from this, the impregnating composition owing to the adhesives contained therein imparts to the base material the necessary adhesive capacity while the material is applied to the type or type plate under 25 pressure, forcing the projecting portions of the type plate or the like into the material of the matrix.

When the impregnating composition has been admixed from the beginning to the material of 30 the matrix as described, the impregnation of its face, or faces, is obviously dispensed with.

The coating composition must possess a partly metallic character and considerable resiliency, and we therefore incorporate therein metals of 35 high melting point ground to extreme fineness, for instance, bronze powder in combination with fillers and binders. A suitable coating compound has the following composition:

|                                    | Parts. |
|------------------------------------|--------|
| 40 Water                           | 500    |
| Metal powder of high melting point | 50     |
| Casein                             | 35     |
| Mineral powder                     | 400    |
| Wax                                | 10     |
| 45 Glycerine                       | 10     |
| Nitric acid                        | 1,5    |
| Alcohol                            | 20     |

The coating composition is applied to the matrix base in cold or hot condition by any suitable process. It may be brushed or sprayed onto the impregnated face, or faces, of the matrix. Obviously the coating layer must be of uniform thickness and of uniform fineness. The finished matrix has a surface which is perfectly smooth and 50 homogeneous and has a metallic lustre. The finished matrix is ground and polished and in this condition is equal to a metal plate, with a perfectly clear and fine reproduction of the original. The 55 same clearness is imparted to the stereotype plates which are cast, or the negative matrices which are molded, from such matrix. The coating composition, particularly on account of the addition of metallic constituents of high melting point, imparts to the matrix almost metallic hardness after the matrix has been dried, but when the matrix is moistened it becomes again ductile and rubber-like so that owing to its plasticity impression is effected in a very short time, about a minute, in 60 cold condition and at a comparatively low pres-

sure. Notwithstanding this softness of the matrix, it retains a very clear and well defined impression while on the other hand the type or other original for which the matrix has been molded, is not worn by the soft and plastic material.

In order to conserve the valuable matrix and to protect it against damage during impression we may insert a metal foil, for instance, aluminium foil, between the back of the matrix and the usual backing of felt or fabric which prevents impression of the texture of the backing into the moist matrix.

A matrix which has been prepared in accordance with our invention is very durable and possesses all properties required for rendering it perfectly resistant to the high temperature of stereotype-plate casting so that it will stand the casting of a practically unlimited number of stereotype plates by automatic rapid casting machines for rotary printing machines.

The matrices are suitable for autotypes from the finest screens which are reproduced in all the clearness and fine definition of the original.

We wish it to be understood that we do not desire to be limited to the exact details of construction shown and described for obvious modifications will occur to a person skilled in the art.

We claim:

1. The process of manufacturing matrices for printing purposes, consisting of a base plate and a coating composition, comprising treating mechanically the surface of said plate so as to render it smooth and uniform, impregnating the mechanically treated surface of said plate with a composition containing a filler for the pores of said base plate, and an adhesive, applying a coating to said treated and impregnated surface, allowing said coating to become dry, and mechanically treating the finished matrix so as to render it smooth and uniform.

2. As a new article of manufacture, a matrix for printing purposes, comprising a base of fibrous material, impregnated with a mixture of an adhesive, a water-repellent material and a metal powder and coated with a mixture of a plasticizer, a water-repellent material, finely divided metal of high melting point and a mineral filler.

3. As a new article of manufacture, a matrix for printing purposes, comprising a base of fibrous material, impregnated with a mixture of an adhesive, a water-repellent material and a metal powder and coated with a mixture of casein, wax, metal bronze and mineral powder in the proportion of 3.5:1:5:40.

4. The process of manufacturing matrices for printing purposes, consisting of a base plate and a coating composition, comprising admixing to the material of the matrix an impregnating composition containing a filler for the pores of the material and an adhesive, molding a base plate from said material, treating mechanically the surface of said plate so as to render it smooth and uniform, applying a coating to said treated and impregnated surface, allowing said coating to become dry, and mechanically treating the finished matrix so as to render it smooth and uniform.

RICHARD JUNGHÄNEL.  
HANS GROSS.

80

85

90

95

100

105

110

115

120

125

130

135

140

145